

July 15, 1941.

E. J. HOUDRY

2,248,994

COMBUSTION OF CARBON MONOXIDE

Filed April 4, 1939

2 Sheets-Sheet 1



INVENTOR  
EUGENE J. HOUDRY  
BY  
Ira d. Nickerson  
ATTORNEY

July 15, 1941.

E. J. HOUDRY

2,248,994

COMBUSTION OF CARBON MONOXIDE

Filed April 4, 1939

2 Sheets-Sheet 2



Fig. 4.

INVENTOR  
EUGENE J. HOUDRY  
BY

Ira L. Nickerson  
ATTORNEY

## UNITED STATES PATENT OFFICE

2,248,994

## COMBUSTION OF CARBON MONOXIDE

Eugene J. Houdry, Ardmore, Pa., assignor to  
 Houdry Process Corporation, Wilmington, Del.,  
 a corporation of Delaware

Application April 4, 1939, Serial No. 266,010

11 Claims. (Cl. 23—2)

This is a substitute for and continuation-in-part of my copending application Serial No. 78,542 filed May 8, 1936.

The invention relates to chemical reactions and more particularly to the oxidation or combustion of carbon monoxide and other burnable material in a gaseous stream.

One object of the invention is to add energy to a gaseous stream. Another object is to raise the temperature of a gaseous stream. Another object is to eliminate toxic, explosive, and incompletely oxidized components of a gaseous stream. Still another object is to devise suitable apparatus for carrying out the above objects. Still other objects will be apparent from the detailed description which follows.

The invention involves the addition of heat to a gaseous stream, such as gaseous mixtures including fumes or waste gases from a combustion, catalyst regeneration, or other zone, by effecting oxidation of CO and other burnable material. If the gases are at a suitable high temperature, as above 1000° F. and oxygen is present, the combustion may be effected in the presence of mere spreading material. If it is desirable to operate at a temperature somewhat below 1000° F., a catalytic agent which will supply oxygen may be utilized. If an oxidizing medium such as air is added to the waste gases, the reaction can be carried on at a still lower temperature. The gaseous stream, when below reaction temperature, is preferably brought thereto by passing it in heat exchange relation with the contact mass or catalytic agent. If air or other oxidizing medium is added to the gaseous stream, care must be exercised to supply it in amounts below the requirement for an explosive mixture. When the gaseous stream contains hydrocarbon vapors and their elimination is important, a highly porous contact mass should be utilized which will withstand the operating temperature and which will retain the vapors by absorption and/or adsorption until burning is effected through the action of the oxidizing agent.

While the invention is capable of rather general application, it is of special importance in connection with the treatment of regeneration fumes from catalytic converters and such a use is indicated in the copending application of myself and R. S. Vose, Serial No. 58,858, filed January 13, 1936 which issued August 1, 1939 as U. S. Patent 2,167,655.

In order to illustrate the invention, concrete embodiments of apparatus, capable of practising

it, are disclosed in the accompanying drawings, in which:

Fig. 1 is a vertical sectional view through a small unit, the section being made substantially on the line 1—1 of Fig. 2;

Fig. 2 is a transverse sectional view substantially on the line 2—2 of Fig. 1;

Fig. 3 is a fragmentary or left half section of Fig. 1, showing a modification; and

Fig. 4 is a vertical, sectional view with certain parts shown in elevation of a different and larger combustion unit.

The apparatus unit illustrated in Figs. 1, 2 and 3 is intended to take care of a gaseous stream of relatively small volume. It provides a reaction zone for the contact or catalytic oxidation mass M, defined by a tubular member 5 having screw-threaded connection with a lower header 6 and welded to an upper header member 7. An outlet pipe 8 leads from the upper end of the reaction chamber for the discharge of the neutral heated fumes which are conducted away to suitable apparatus diagrammatically indicated at 9 for utilization of kinetic or heat energy in the gaseous stream.

The gaseous material to be treated may enter the lower end of the reaction zone by an inlet pipe 10 extending through header 6. To insure the stream entering the zone at the proper temperature and also to give a measure of control of the reaction through removal of at least a portion of the heat of reaction, the stream, prior to its admission to pipe 10, is brought into extended heat exchange with the reaction zone, but such heat exchange is confined, primarily, to radiation. By preference, the gaseous stream picks up heat progressively as it is caused to traverse the length or depth of the reaction zone. In Figs. 1, 2 and 3, the heat exchange is effected upon the exterior of the reaction zone. As indicated, feed conduit 11 is formed in a coil 11a which encircles the reaction zone throughout its length from outlet end 8 to inlet end 10. The turns of coil 11a may be maintained in definite spacial relation to tubular wall 5 of the reaction zone by suitable members such as rods or posts 12 (Figs. 1 and 2) which may be inserted through holes or bores 12a in upper header 7, while the opposite ends are received in sockets 12b in lower header 6. A wire, cotter pin, or other member is inserted through the rods as at 12c to retain them in place. To control the quantity of heat absorbed by the feed per unit of length of the reaction chamber, and to provide for expansion of the stream, coils 11a may be increased in size

as they approach inlet 10, this increase being effected in stages by the use of sections of pipe of increased diameter, or gradually and progressively as indicated in Fig. 1. The lower end of coil 11a is joined to inlet conduit 10 by a suitable connection 13. To prevent loss of heat from the unit, an outer casing 14, which is preferably in sections to allow for the pipe connections 11 and 13, is secured to upper and lower headers 7 and 6 in any suitable manner, as by seating the lower end in an annular recess 6a in lower header 6, while the upper end is attached or clamped to header 7 as by a split ring 15. A layer of heat insulating material 16 may be applied to the entire exterior of the unit.

Progressive pickup of heat by radiation may be effected between the feed and the reaction zone in other ways. If it is not desired to increase the size or diameter of the conduit making up coil 11a, a conduit of uniform diameter may be utilized, but the pitch of the coil may be decreased as lower header 6 is approached by making the coils closer together, thereby increasing the radiating surface. If uneven spacing of the coils is objectionable, the same effect of progressive heat exchange may be secured by attaching plates of different sizes indicated at 17 (Fig. 3) to the conduit coils 11b, as by welding.

If such a large volume of gas must be treated that the type of unit shown in Figs. 1 to 3 is unsuitable, a different unit, such as shown in Fig. 4, may be utilized. This unit comprises a central cylindrical member 20 having end closures 21 and 22 and upper and lower partitions or flue sheets 23 and 24 dividing the interior of the case into a large central reaction chamber to contain the contact mass or catalyst M and end manifolding chambers 25 and 26. Assuming that the gaseous stream enters the manifolding chamber 25, it is brought into heat exchange with mass M through suitable perforated heat exchange and distributing members 27 embedded in the mass. They may be supported by upper partition 23 and extend substantially through the reaction chamber. One of these members (the central one) is shown in section and comprises an inner conduit 27a which communicates through partition 23 with manifolding chamber 25 on the one hand and discharges the gas at the very bottom of the outer conduit 27b which is spaced from and encloses the inner conduit. Outer conduit 27b has perforations throughout its length for discharging the gaseous material at reaction temperature directly into contact mass M. To insure a substantially even pickup of heat by the gaseous stream from the contact mass as it passes through inner conduit 27a, suitable heat baffling means, such as baffle members 27c and 27d of different length are provided. Instead of sheet metal baffles, such as indicated, heat insulating material may be utilized as a substitute for or in combination with such baffles, as indicated, for example, in U. S. Patent No. 1,987,636, issued January 15, 1935 to T. B. Prickett and myself, and in U. S. Patent No. 1,987,933 issued January 15, 1935 to J. W. Harrison. The gases, after being distributed uniformly at substantially even temperature all through mass M, may pass therefrom through suitable perforations in partition 24 into outlet manifolding chamber 26, or may be withdrawn uniformly from all parts of the mass by perforated conduits such as 28 embedded in the contact mass in symmetrical arrangement and in parallelism with the distributing and heat exchange members 27 to effect a parallel flow of the gaseous

fluid through the mass, such conduits extending through partition 24 to communicate with manifolding chamber 26. The entire casing is lagged with heat insulating material as indicated at 29, and, in addition, the inner walls of inlet manifolding chamber 25 are lined with a layer 25a of heat insulating material.

In the apparatus units illustrated in the drawings, it is apparent that the gases to be oxidized are passed through the conduits in radiant heat exchange with the walls which define the reaction chamber and which enclose the catalytic or other contact mass, and that provision is made to increase the temperature of the reactants by increased surface areas, by baffles, or by other means so as to remove substantially equal amounts of heat from all parts of the reaction zone. When very large quantities of heat are liberated within the converter the cooling effect of the entering reactants may be supplemented by extraneous heat exchange fluid which may optionally be mixed with the entering reactants or sent through the reaction zone in suitable conduits as indicated for example in the aforesaid Harrison Patent No. 1,987,933 or in Patent No. 2,078,947 issued May 4, 1937 to myself and R. C. Lassiat.

One reaction to which the process is particularly adapted is in the combustion of carbon monoxide and/or oil vapors which may be present in regenerating fumes issuing from a catalytic converter for the purpose of increasing the energy content of the fumes, which may be thereafter recovered either as kinetic energy or as heat energy or both, as indicated, for example in the aforesaid copending application of myself and R. S. Vose. The combustion is best effected when a contact mass is employed. The mass may vary in character, depending upon the temperature at which the gaseous stream enters the combustion chamber. When it enters at high temperatures, as of the order of 1000° F. or more, and containing sufficient oxygen, the contact mass may be mere inert spreading material, but preferably of a highly porous nature, so as to retain oil vapors and the like until combustion is effected, such as pumice, kaolin, firebrick, and other blends of silica and alumina. This material is preferably in the form of lumps, fragments, or molded pieces.

When the gaseous stream enters the combustion zone at a temperature below 1000° F., as of the order of 900° F., the contact mass may comprise or contain catalytic material, such, for example, as metallic oxides and compounds, including those of copper, iron, cobalt, nickel and lead. The metals may be utilized directly, as in the form of shavings or turnings, or the metal or metallic compound may be in finely divided form on or incorporated in suitable supports such as inert or active blends of silica and alumina of natural or artificial origin, preferably in the form of lumps, fragments, or molded pieces. If the operation is to be effected with initial temperatures much below 900° F., as of the order of 700° F., it is sometimes desirable to add air or other oxidizing medium to the fumes. This medium should be added in amounts below that which will give an explosive mixture with the carbon monoxide and other burnable material which may be present in the gaseous stream. For fumes from the regeneration of catalytic material in a converter utilized for the conversion or treatment of hydrocarbons, up to about 6% of air is suitable. This may be added before the stream

is brought into heat exchange with the reaction zone, as, for example, by branched pipe 30 (Figs. 1 and 4). Other fluids, such as non-explosive fuel or extraneous cooling fluid such as atomized water, inert gas, etc. may be added at this point to control the entering and exit temperature of the gaseous stream. A more preferable point of admission of air is just before the gaseous stream enters the reaction zone, as by branched pipe 31 (Fig. 1). However, the oxidizing medium can be admitted at either point in Figs. 1 and 2, or in fractional amounts at both points.

If kinetic energy is to be recovered from the fumes by the use of a turbine or other heat or expansion engine capable of supplying motive power, the maximum operating temperature of the fumes is of the order of 950° F. In that case, the fumes may enter the reaction chamber at about 750° F. under pressure and the rate of heat removal from the chamber regulated to provide a temperature rise of the fumes of about 200° F. For heat recovery purposes, higher temperatures in the fumes could be utilized, as up to 1200° F., but such high temperatures would require the use of alloy or other special steels in the combustion unit to stand such temperatures.

The rate of feed of the gaseous stream and of any other cooling fluid to the combustion zone is adjusted to attain a wall temperature such that no part of the contact mass is cooled below predetermined and preferably substantially constant operating or oxidizing temperature. Hence rates of feed will vary with different ratios of heat exchange surfaces to volume of catalyst. There is also a tendency to increase feed rates with decreased concentrations of burnable material. Rates up to 60:1 (sixty volumes of charge to one volume of contact mass) per minute have been used. A good rate for a gaseous stream supplied at 520° F. and containing about 2% CO by volume and .2% hydrocarbons by weight is about 13:1 in a reaction chamber having a contact mass volume to heat-exchange-surface area of about 1:16, the mass comprising hydrosilicate of alumina with copper oxide content of about 15% by weight. The operation gives a final or outlet temperature of about 920° F., thus providing increase in temperature of the gaseous stream of about 400° F.

Theoretically, to oxidize 1 pound of oil or other similar burnable material, 3½ pounds of oxygen are required which can be provided by 14 pounds of copper as copper oxide (CuO) based on complete reduction of CuO to Cu; and to oxidize 100 cubic feet of CO there is required 4.25 pounds of oxygen which can be supplied by 17 pounds of copper. When oxygen is present or is added to the stream, smaller quantities of catalyst or oxidation promoter may be used. In practice, it is advisable to supply a large excess of oxidation promoter, as five to ten times the theoretical amounts, to insure a sufficient amount of active material, thus providing for (a) variations in the composition of the gaseous stream, (b) channelling of the mass, (c) progressive poisoning by formation of sulphates, and (d) incomplete reduction of the oxide to metal. Relative amounts of the listed metals other than copper may be utilized, some regard being given to their atomic weights and to the molecular weights of their oxides.

The maximum amount of oxidation promoter which can be used in a given volume of space is dependent upon the rate at which heat can

be removed by suitable heat exchange surfaces. Hence, when the contact mass is a poor conductor of heat, such as a silica-alumina blend, it has been found desirable to incorporate therein only a restricted amount of the promoter, as not more than 15% by weight of the mass, by reason of the sharp rise in temperature which occurs when the promoter is reoxidized.

The combustion reaction is effected equally well under pressure or without pressure. When kinetic energy is recovered, the addition of atomized water, cool gas, and the like under pressure at branch 30 in advance of the heat exchange zone is of importance not only as a means of temperature control of the reaction zone, but also as a means of increasing the recoverable energy of the gaseous stream. In most instances, the gaseous stream which is fed to the combustion zone will contain sulphur compounds of some kind, such as H<sub>2</sub>S, SO<sub>2</sub>, SO<sub>3</sub>, etc., which are removed from the gaseous stream in combining with the promoter to form sulphates, thereby producing a gradual poisoning of the catalyst while the latter purifies the gaseous stream of its corrosive or sulphurous constituents. Hence regeneration will be required from time to time at more or less infrequent intervals depending upon the composition of the gaseous stream and upon the quantity of metallic oxide in the contact mass. Regeneration is by reduction, and hydrogen, or a hydrogen carrier such as refinery gas, may be utilized.

Of the metallic oxides mentioned above, copper oxide was found to give the best result and to promote oxidation for the longest period. It is the only one which acts when no oxygen is present in the gaseous stream, but this oxide must be at relatively high temperature, good results being obtained for example at about 900° F. When used in suitable amount, copper oxide is capable of supplying oxygen for combustion for the burning of oil vapors and carbon monoxide when there is little or no oxygen present in the gaseous stream, as, for example, during the early stages of regeneration of catalytic material. The copper catalyst easily regains its oxygen, and is reconverted to copper oxide, as during the latter stages of a regenerating period, when substantial amounts of oxygen are unused during the regeneration and are accordingly present in the gaseous stream. When small amounts of air are admitted to the gaseous stream, as up to 6%, the copper catalyst functions efficiently at temperatures of about 700° F. All CO and other burnable material is consumed, and the resulting fumes are inert and hence capable of utilization where material of this character is needed. One use is as a purging agent for catalytic masses, as, for example, when other purging agents, such as steam, are not available or cannot be used. It can also be used as vaporizing or other process fluid, and for repressuring of converters after vacuum purging operations.

Apparatus aspects of the invention are claimed in my copending divisional application Serial No. 255,459, filed February 9, 1939.

I claim as my invention:

1. The process of producing a stream of substantially inert fluid of controlled recoverable energy content comprising the steps of passing through a combustion promoter maintained under combustion conditions a stream of fumes resulting from burning of organic deposit formed on a contact mass and containing CO and suspended unburned organic material, regulating

the temperature of the combustion promoter and of the stream of burned gases issuing therefrom and from the reaction zone at predetermined and substantially constant level within the range of 700 to 1200° F., and effecting such regulation at least in part by absorbing excess heat of combustion in a stream of extraneous cooling fluid passed in indirect heat exchange relation with the combustion zone.

2. In the treatment of regeneration fumes containing burnable components including carbon monoxide and resulting from removal of burnable deposits from contact masses, the process of passing a stream of such fumes through a combustion zone containing a combustion promoter maintained under combustion conditions to convert such burnable components into inert fluid and to increase the available energy content of said fumes, and maintaining the stream of inert gases issuing from said zone at predetermined and substantially constant temperature below 1200° F. by transferring heat of combustion from said zone to said fumes before entry of said fumes to said combustion zone.

3. In the production from combustion gases containing burnable components including carbon monoxide and resulting from combustion of burnable deposits in contact masses of an inert process fluid of controlled energy content valuable for supplying industrial energy, the process of subjecting a stream of said gases to promoted burning in a combustion zone to convert said burnable components into inert fluid, absorbing excess heat of reaction from said combustion zone at regulated rate by an extraneous heat exchange fluid to limit to a maximum of 400° F. the temperature increase of said gases in traversing said zone and to maintain predetermined and substantially constant temperature below 1200° F. in the stream of inert process fluid resulting from the combustion and issuing from said zone.

4. In the treatment of regeneration fumes containing burnable components and formed by burning combustible deposits from contact masses, the process of producing a stream of inert fluid valuable for supplying motive power comprising subjecting a stream of such fumes to promoted combustion with the aid of a contact mass containing a metal or metal oxide combustion promoter to convert said burnable components into inert fluid, maintaining the stream of burned fumes issuing from said mass at substantially constant temperature not in excess of 950° F., and regulating the temperature of said burned fumes by absorbing excess heat of combustion in an extraneous cooling fluid passed in direct heat exchange relation with said mass.

5. In producing valuable process fluid from combustion gases containing burnable components including carbon monoxide, the process of sending a stream of such gases under combustion conditions into and through a reaction zone containing a contact mass capable of promoting combustion of said burnable components, admitting a stream of said gases at substantially uniform temperature to said mass at a multiplicity of points distributed within and throughout the same, maintaining said mass at substantially constant temperature below 1200° F. so that the stream of burned inert fumes issuing therefrom are at substantially constant, predetermined industrially practical temperature, and effecting such temperature control by passing said gases diluted with an extraneous cooling

fluid in heat exchange relation with said reaction zone before admitting them to said mass.

6. The process of treating regeneration fumes containing burnable components and resulting from removal by combustion of burnable deposit from contact masses contaminated by the same comprising the steps of subjecting a continuous stream of said fumes while still hot to controlled combustion with the aid of a contact mass containing a combustion promoter to convert said burnable components into inert fluid and to produce a stream of process fluid of regulated energy content, admitting said fumes at substantially uniform temperature to a multiplicity of points within and throughout said mass, simultaneously passing an extraneous cooling fluid in heat exchange relation with said mass to remove excess heat of reaction therefrom and to maintain substantially uniform temperature within and throughout the same, and regulating absorption of reaction heat from said mass to provide predetermined and substantially constant temperature below 1200° F. in the burned fumes issuing from said mass.

7. The process of preparing for industrial use regeneration fumes containing burnable components including carbon monoxide issuing from a catalytic converter comprising the steps of sending a stream of such fumes at temperature in excess of 500° F. into a reaction zone containing a contact mass capable of promoting combustion of said burnable components, regulating reaction conditions through absorption of combustion heat therefrom to limit temperature increase of the fumes during their passage through said zone to a maximum of 400° F. and to provide delivery of burned fumes from the zone at substantially constant temperature below 1200° F., effecting at least a portion of said heat absorption by passing the unburned fumes in indirect heat exchange relation with said mass, and maintaining substantially uniform temperature in said mass by progressively increasing radiant heat exchange between the zone and said unburned fumes, and by admitting the heated fumes at substantially uniform temperature to the mass at a multiplicity of points distributed within and throughout the same.

8. In the treatment of fumes made during regeneration by burning from contact masses carbonaceous deposit formed when the mass assists organic reactions, said fumes containing CO, hydrocarbons and quantities of oxygen varying from insufficient to excess, the process comprising passing a stream of said fumes under combustion conditions through a single combustion promoting mass made up of a minor quantity of copper oxide in finely divided form distributed on a porous inert support which holds and retains unburned material suspended in said fumes, and maintaining said mass at substantially constant temperature within the range of 700 to 1200° F. by simultaneously passing said fumes and an extraneous heat exchange fluid in heat exchange relation therewith, whereby a stream of inert gases substantially free of burnable components suitable for industrial use issues from said mass at substantially constant and predetermined temperature, said mass supplying oxygen to the combustion reactions during periods of oxygen deficiency in the fumes and regaining a supply of oxygen for this purpose during later periods when the regeneration fumes contain excess unused oxygen.

9. The process of producing inert gas of con-

trolled heat content from fumes containing CO, hydrocarbons and varying quantities of oxygen and resulting from a period of regeneration by burning of carbonaceous deposit from a contact mass wherein said fumes are deficient in oxygen early in the regeneration period and later contain excess unused oxygen, comprising the steps of continuously passing a stream of said fumes through a combustion promoting mass made up of copper oxide in finely divided form distributed on a porous support which holds and retains unburned material suspended in said fumes, and maintaining said mass at substantially constant temperature not over 1000° F. by passing said fumes in heat exchange relation with said mass while simultaneously utilizing a stream of extraneous cooling fluid to assist the fumes in removing excess heat of reaction from the mass, whereby the stream of inert gases continuously issues from the mass at predetermined, substantially constant temperature and said copper oxide supplies oxygen to the combustion reactions early in the regeneration period and later in that period regains a supply of oxygen.

10. In the treatment of fumes made during regeneration by burning from contact masses carbonaceous deposit formed when the mass assists organic reactions and containing CO, hydrocarbons and quantities of oxygen varying from excess to deficiency, the process comprising passing a stream of said fumes under combustion conditions through a single combustion promoting mass made up of about 15% by weight of copper oxide in finely divided form distributed on a porous support of a blend of silica and alumina, maintaining said mass at substantially constant temperature in the range of 700 to 1200° F. by passing said fumes diluted with a

- controlled amount of an extraneous cooling fluid in indirect heat exchange relation therewith, whereby a stream of inert gases substantially free of burnable components suitable for industrial use issues from said mass at substantially constant and predetermined temperature, said catalyst supplying oxygen to the combustion reactions during periods of oxygen deficiency in the fumes and regaining a supply of oxygen for this purpose during later periods when the regeneration fumes contain excess unused oxygen.
11. The process of producing inert gas of controlled heat content from combustion fumes containing CO, hydrocarbons and amounts of oxygen varying from excess to deficiency and resulting from a period of regeneration by burning of sulphur bearing carbonaceous deposit from a contact mass comprising the steps of passing a stream of the regeneration fumes at temperature in excess of 500° F. and under combustion conditions through a contact mass made up of an active metal oxide combustion promoter and desulphurizing agent distributed in finely divided form on a porous siliceous support, regulating the temperature of said mass by simultaneously passing said fumes and an extraneous heat exchange fluid in indirect heat exchange relation therewith to maintain the same at substantially constant temperature below 1200° F. and to limit temperature increase of the fumes during their conversion into inert gaseous form to a maximum of 400° F., and periodically passing reducing fluid through said mass to reduce to oxide form metallic sulphate formed in the mass as a result of sulphur removal under combustion conditions.

EUGENE J. HOUDRY.

CERTIFICATE OF CORRECTION.

Patent No. 2,248,994.

July 15, 1941.

EUGENE J. HOUDRY.

It is hereby certified that error appears in the printed specification of the above numbered patent requiring correction as follows: Page 4, first column, line 57, claim 4, for the word "direct" read --indirect--; and second column, line 54, claim 8, for "insufficient" read --insufficiency--; page 5, second column, line 7, claim 10, for "catalyst" read --mass--; and that the said Letters Patent should be read with this correction therein that the same may conform to the record of the case in the Patent Office.

Signed and sealed this 26th day of August, A. D. 1941.

Henry Van Arsdale,  
Acting Commissioner of Patents.

(Seal)